

Nov. 13, 1951

C. N. HICKMAN

2,574,479

PROPELLANT HAVING AN OPACIFIER FOR PREVENTING  
SELF-IGNITION BY RADIANT ENERGY RADIATIONS  
Filed Jan. 30, 1943



INVENTOR  
CLARENCE N. HICKMAN

BY  
C. E. Herestrom & H. F. Shilcock  
ATTORNEYS

## UNITED STATES PATENT OFFICE

2,574,479

PROPELLANT HAVING AN OPACIFIER FOR  
PREVENTING SELF-IGNITION BY RADI-  
ANT ENERGY RADIATIONSClarence N. Hickman, Jackson Heights, N. Y., as-  
signor to the United States of America as rep-  
resented by the Secretary of War

Application January 30, 1943, Serial No. 474,213

1 Claim. (Cl. 52—13)

(Granted under the act of March 3, 1883, as  
amended April 30, 1928; 370 O. G. 757)

1

The invention described herein may be manufactured and used by or for the Government for governmental purposes, without the payment to me of any royalty thereon.

This invention relates to jet propulsion devices and to propellants therefor, and has for its principal object the provision of a propellant which, when burned under the conditions existing in a rocket combustion chamber, will produce a pressure-time curve which can be controlled and predicted by the initial form and dimensions of the powder.

The principal object of this invention can be achieved only when the propellant which is used possesses, during the major portion of the burning, a closely defined burning surface which varies in accordance with the law of burning by uniform layers. This requires that the burning take place only on the surfaces exposed by the burning away of the outer layers, and that there be no additions to the burning surfaces such as those produced by internal burning or the breaking away of the outside surfaces.

Since the propellant burns only on its exposed surfaces, the rate of gas evolution, and the pressure developed, will depend at any instant upon the area of the burning surface. The initial burning surface will depend upon the form and dimensions of the grain. If as the burning continues, there is an increase in the effective burning area for any reason, this increased area upon burning will evolve gas at a higher rate thus producing a higher pressure. I have found that a pressure-time curve of the desired shape can be obtained by the use of a grain form such that the curve of the burning area against time is substantially similar in shape, during equilibrium burning, to the shape desired in the pressure-time curve.

It, therefore, becomes another object of this invention to provide a rocket propellant in the form of a powder grain having a substantially constant burning surface throughout the burning time.

In order to accomplish the above object I prefer to use a cylindrical stick of powder having a single concentric cylindrical perforation formed therein.

One of the most suitable propellants from the point of view of energy, content and availability is a so-called "double-base" powder. These double-base powders are formed into "grains" by any one of several well known methods, which need not be described herein.

The motor weight restrictions in a jet propelled

device, such as a rocket, place rather severe limitations on the burning characteristics of propellants. They must, after ignition, burn evenly and uniformly with time, under the pressure conditions existing in the chamber, without developing pressures exceeding the allowable limit for the chamber in which the propellant is disposed. The pressure developed in the motor chamber should remain fairly constant or increase slightly so that the propellant will burn completely, but, as stated, the pressure must not increase to high values. If the latter should happen, the motor chamber walls may burst. If such failure occurs in the projector tube during the firing of the rocket, the tube itself may burst. Increases in pressure during burning after the rocket has left its projector tube may burst the motor chamber. Either type of bursts results in hazards to the firing personnel and equipment.

To provide a propellant in which the burning area may be regarded as constant, I utilize a cylindrical stick of powder having a single cylindrical axial perforation and space the powder grain from the inner walls of the combustion chamber so that the inner and outer cylindrical surfaces may be exposed for burning. The burning surface area of a cylindrical stick of powder having a concentric cylindrical perforation may be regarded as constant only if the burning surface area of the ends is neglected. The ends can be neglected when the length of the stick is large compared to the diameter. If, however, the length of the stick is short the degressive effect due to burning at the ends may be great. In order to overcome this disadvantage the ends may be treated with a material which will inhibit combustion. A material which I propose is tar. If the ends are painted with tar the burning area will be constant, and substantially constant pressures will be maintained. Other inhibitors such as cellulose acetate or rubber compounds could be used.

In the course of my researches on the use of large grains of double-base, translucent powder for rocket motors and other like jet-propelled devices, I discovered that such grains almost always developed abnormally high pressures during burning in the rocket motor. I used translucent grains because any cracks or flaws therein which produce a non-uniform burning surface may thus be determined by visual inspection prior to loading in the combustion chamber. Translucent grains consisting of cylindrical tubes of about  $\frac{1}{8}$  inch outside diameter and  $\frac{1}{4}$  inch inside diameter

55 appeared to be uniform throughout, no holes,

cracks, areas of uneven colloiding, or fibers of nitrocellulose being observed. Such a powder grain would have been expected to give superior results as a propellant powder in a rocket. Yet, as stated, failures were common. Pressures developed during burning would be so high as to break the stick into pieces and to expel partially burned pieces of powder from the rocket motor.

I was finally able to examine partially burned powder, and to subject such powder grains to partial burning tests, using apparatus as described in my copending application S. N. 501,002, filed Sept 2, 1943, now matured to U. S. Patent No. 2,464,179. I discovered that partially burned, light translucent powder grains had surfaces marked by fissures, "worm holes" and even cracks. These fissures were frequently of substantial depth and area. Thus it was apparent why the pressure increased, frequently by several thousand pounds, during burning. For some unknown reason the translucent powder fissured during burning, the fissures formed resulted in increased burning area and, as a consequence, in excessive increases in pressure.

The increase in pressure, sometimes exceeding the bursting strength of the motor chamber, is a kind of progressive process. That is to say, when a small fissure or worm hole forms, the burning surface of the powder grain is slightly increased. This leads to an increased volume of gas, which in turn increases the pressure in the motor chamber. The increase in pressure increases the rate of burning, more fissures form, again increasing the pressure with further increase in burning speed so, in a fraction of a second, the propellant, instead of burning evenly, burns with explosive force and the development of very high pressures in the motor chamber.

On the other hand, when fissuring is prevented, in accordance with my invention, the powder grains of my invention burn smoothly from the surfaces inwardly, and the burning rates, pressures developed, etc., can be correlated with the structural design of the rocket motor chamber, nozzle area, etc.

Many explanations of the cause of fissuring were advanced. A "shock wave" theory was proposed, and ultimately discarded. Others attributed it to some peculiarity in the physical structure of the powder grain, i.e., its brittleness.

I finally hit upon an explanation based on radiation phenomena. I felt that as the surfaces of the powder burned, the light energy developed was radiated below the burning surface into the interior of the grain where selective ignition of nitroglycerin molecules could possibly occur. If that happened it would be reasonable to believe that the combustion products "wormed" through to the surface of the grain, thus creating channels or fissures, and exposing more surface area where burning would take place. This radiation explanation then led me to the conclusion that the powder grain should not be translucent, and further led to the discovery that opacifiers could be incorporated in the powder grain to render the grain opaque to light rays which appear to be the cause of fissuring.

As a result of my discoveries I am able to provide a double-base propellant for jet propulsion devices which performs satisfactorily under the conditions imposed by the thin walls of the combustion chamber utilized in such devices. My invention is thus based in part on the discovery that a propellant for a rocket should have a configuration producing a constant area of burning

and that double-base propellants for use in rockets and like jet propelled devices must be opaque to the light rays which appear to cause fissuring.

It should be understood, however, that there may be applications in rocket propulsion wherein configurations other than that disclosed may be desired to produce for example a slightly progressive powder to reduce burning time. However, in these specific instances it is still important that an opaque powder grain be used in the rocket chamber to prevent fissuring which if occurring would disrupt the calculated burning time and produce pressures higher than those which the rocket combustion chamber was designed to withstand.

In order that my invention may be more clearly understood, I have, on the appended single sheet of drawings, illustrated a powder grain of cylindrical configuration, having a single axial cylindrical perforation formed therein, so that when burned on both surfaces it will offer a substantially constant burning area. The surface of the propellant shown in one view has developed fissures and worm holes after partial burning. It has also been noted that the worm holes which do not extend to the surface are observable within the interior of the grain. This will more clearly illustrate what is meant by terms "worm holes" and "fissures." I have also shown a schematic representation of a rocket device containing the propellants of the present invention.

In the drawings—

Fig. 1 is a powder grain of the present invention;

Fig. 2 shows a powder grain which has fissured, and

Fig. 3 is a representation of a rocket containing the opaque propellants of my invention.

In Fig. 2 the grain 1 has its surface marked and scored by fissures 10 and worm holes 2. This grain is translucent to light.

In Fig. 1 the grain 3 shows no fissuring after partial burning. This grain is opaque to the light rays.

In Fig. 3 the rocket motor chamber 4 is provided with plurality of cylindrical sticks of opaque powder 3, each of which has a single axial cylindrical perforation 6, and which, if of small diameter compared to their length, have their end surfaces painted with tar. The propellant sticks are held in place by the trap wires 7 threaded through the perforations 6. For purpose of clarity of illustration these grains are shown spaced from each other, although this is not generally carried out in practice. The nozzle or venturi of the motor is shown at 8 and the "pay load" or high explosive head at 9.

The present invention, therefore, comprises the use of a propellant in a rocket chamber, said propellant being characterized by the fact that it is opaque, and also by the fact that it differs from the propellants originally tried but which were found to be unsatisfactory since they produced fissures and excessive pressures, only in that it is opaque; whereas the other propellants referred to were translucent. I prefer to make the propellant opaque by the addition of a suitable opacifying agent.

This invention also includes the combination of a rocket motor combustion chamber and propellant which has the form of a cylinder with a single concentric cylindrical perforation formed therein; the configuration retains during burning a constant surface area. In the case of short

grains or in other cases where a more exactly constant burning area is desired, the invention may include the treating of the end surfaces with an inhibitor such as tar.

This invention also includes the combination of a rocket motor combustion chamber and propellant having the opaque character stated, but not limited to any specific geometrical configuration. For the propellants involved in this invention I prefer to use the double-base powder.

By double-base powder or propellant I mean any mixture of nitrocellulose and nitroglycerin in those proportions which will give propellant characteristics. Such proportions are well known in the art and I need not elaborate on them in this specification. As a rule the nitrocellulose exceeds the amount of nitroglycerin, but propellants containing equal quantities of such constituents have been made and are useful. I do not wish to be limited to any particular proportion of nitrocellulose and nitroglycerin, since my invention does not depend upon such proportions. Likewise, the amount of opacifier to be incorporated in the mixture for the purpose stated can vary over wide limits. The final result is a powder which is opaque to light energy which appears to cause fissuring in the absence of the opacifier. The opacifier is quite uniformly distributed throughout the powder grain. In the case of soluble coloring agents, such as nigrosine, the entire grain is colored. In the case of solid opacifiers such as lampblack or carbon black the finely divided particles thereof are quite uniformly distributed throughout the powder grain, although there may be zones having a higher concentration of the solid; but visual inspection of any surface reveals that the solids are well distributed. Photo micrographs of surfaces produced by cutting the grain at various points, at fairly high magnifications, show the finely divided solid particles scattered more or less uniformly through the body of the powder. Obviously, the use of lampblack, graphite and the like in my invention bears no similarity to the coating or surface treatment of powder grains after they have been formed for the purpose of modifying the burning characteristics of the grain surface.

Those skilled in the art will appreciate that many different opacifiers can be used in the practice of my invention. For example, lampblack is an excellent material to incorporate in the propellant along with the other major constituents. Nigrosine, a black aniline dye, is useful. Any colored, or coloring material, capable of screening out those light rays which appear to cause fissuring, can be used. Thus the desired end may be achieved through the use of dyes, stains or pigments.

Thus a double-base powder containing about 40 percent nitroglycerin, 58 percent nitrocellulose, and 2 percent ethyl centralite is prepared in sheet form for extrusion. This powder, if extruded to grains in the form of cylinders  $\frac{1}{8}$  inch outside and  $\frac{1}{4}$  inch inside diameters will fissure when burned. In the practice of my invention I incorporate about .15 to 0.5 weight percent of lampblack in the powder. The lampblack can simply be rubbed on the sheeted powder before extrusion thereof. When the lampblack coated sheet is extruded the coloring agent is sufficiently dis-

seminated through the grain to render it opaque to light. Alternatively the lampblack can be added to the nitroglycerin prior to colloidizing nitrocellulose.

When using dyes such as nigrosine, not so much opacifier is required. I need only add 0.1 weight percent of nigrosine to the powder constituents to render the final grain opaque. Black p-aminophenol is a suitable opacifier, and there are many others. The object, in each instance, is so to color the final grain that light energy developed on the surface during burning is not permitted to penetrate below the burning surface. This is most easily accomplished by simply coloring the grain throughout with any suitable agent which will inhibit the penetration of the light energy which appears to cause the fissuring. I believe that the red end of the light spectrum is the particular cause of fissuring and therefore coloring agents or "opacifiers" which shield only against the penetration of red rays will be operative. But coloring agents such as carbon black, lampblack, aniline dyes, etc., are so readily available and useful that I find them quite advantageous.

Having thus described my invention, what I claim is:

A propellant grain for jet-propelled devices, comprising a double base powder containing 58% nitrocellulose, 40% nitroglycerin and 2% ethyl centralite, an opacifier consisting of .15 to 0.5 weight percent of lampblack incorporated in said powder, said opacifier being dispersed uniformly throughout the powder to form a composite opaque mixture which will prevent internal self-ignition of the powder by radiant energy radiations produced by surface burning of the powder.

CLARENCE N. HICKMAN.

40

#### REFERENCES CITED

The following references are of record in the file of this patent:

#### UNITED STATES PATENTS

| 45 | Number    | Name       | Date           |
|----|-----------|------------|----------------|
|    | 175,735   | Nobel      | Apr. 4, 1876   |
|    | 328,919   | Chambers   | Oct. 27, 1885  |
|    | 437,499   | Mindeleff  | Sept. 30, 1890 |
|    | 440,921   | Mindeleff  | Sept. 30, 1890 |
| 50 | 1,003,411 | Bales      | Sept. 19, 1911 |
|    | 1,308,343 | Du Pont    | July 1, 1919   |
|    | 1,376,029 | Olsen      | Apr. 26, 1921  |
|    | 1,611,353 | Lepinte    | Dec. 21, 1926  |
|    | 1,709,868 | O'Neil     | Apr. 23, 1929  |
| 55 | 1,788,438 | Norton     | Jan. 13, 1931  |
|    | 1,838,984 | Berkowitz  | Dec. 29, 1931  |
|    | 2,008,889 | Wagner     | July 23, 1935  |
|    | 2,038,700 | Woodbridge | Apr. 28, 1936  |
|    | 2,062,495 | Brayton    | Dec. 1, 1936   |
| 60 | 2,131,354 | Marsh      | Sept. 27, 1938 |
|    | 2,131,383 | Marsh      | Sept. 27, 1938 |
|    | 2,235,298 | Olsen      | Mar. 18, 1941  |
|    | 2,408,252 | De Ganahl  | Sept. 24, 1946 |
| 65 | 2,440,327 | Crawford   | Apr. 27, 1948  |

#### FOREIGN PATENTS

| 70 | Number  | Country       | Date          |
|----|---------|---------------|---------------|
|    | 12,325  | Great Britain | of 1895       |
|    | 15,553  | Great Britain | of 1898       |
|    | 21,482  | Great Britain | of 1903       |
|    | 516,865 | Great Britain | Jan. 12, 1940 |